

Feb. 5, 1929.

1,701,299

E. W. ENGLE ET AL

TANTALUM ALLOY PEN

Filed May 27, 1927

*Fig. 1*



*Fig. 2*



*Inventors:*

*Muner M. Austin and Edgar W. Engle*

*By: Williams, Bradbury, McCaleb & Niblack*

*Atty.s.*

Patented Feb. 5, 1929.

1,701,299

# UNITED STATES PATENT OFFICE.

EDGAR W. ENGLE, OF LAKE FOREST, AND MINER M. AUSTIN, OF WAUKEGAN, ILLINOIS,  
ASSIGNORS TO FANSTEEL PRODUCTS COMPANY, INC., OF NORTH CHICAGO, ILLINOIS,  
A CORPORATION OF NEW YORK.

## TANTALUM-ALLOY PEN.

Application filed May 27, 1927. Serial No. 184,563.

This invention relates to pens and instruments adapted for writing, drawing and the like. More particularly our invention relates to an alloy of tantalum and a metal of the chromium group. We have found that this alloy is especially suitable for this purpose in that the alloy, hereafter defined, retains the hardness, toughness and non-corrosive properties of tantalum, with the increased elasticity, flexibility and resiliency imparted to the tantalum by the addition of the element of the chromium group which is preferably tungsten.

10

Tantalum has been suggested as a suitable metal for making pens, drawing instruments and the like, and considerable experimentation and commercial use has been made of this idea.

To render the tantalum harder, it has been treated with iron, oxygen, hydrogen, silicon, boron, aluminum, titanium, tin, carbon, etc., but none of the proposed treatments has been successful as is evidenced by the fact that tantalum pens are not employed extensively or manufactured on a commercial scale. The hardening substances heretofore used have had a tendency to make the metal so brittle that it could not be successfully worked, and the permissible quantities of these added elements had to be carefully chosen and the additions regulated to a very fine degree.

20

25

30

The object of this invention is to provide a tantalum-alloy pen which will combine the non-corrosive properties, the hardness and toughness of tantalum with pronounced elasticity, flexibility and resiliency by the addition of a metal of the chromium group.

A further object of the invention is to provide a tantalum-tungsten pen with a hardened tip.

35

Other objects will be apparent as the description of our invention proceeds.

In the accompanying drawings which represent preferred embodiments of our invention,

40

Fig. 1 represents a conventional pen made entirely of our tantalum-tungsten alloy, and

Fig. 2 represents an embodiment wherein the shank may be of steel, the nib portion of the tantalum-tungsten alloy, and the point of iridosmium.

45

50

Heretofore alloys of tantalum and tungsten have been very difficult to obtain—espe-

cially alloys in which the tungsten content exceeded two or three percent. By an extensive research on this subject a method for preparing such an alloy has been developed by intimately mixing powdered tungsten with powdered tantalum, compressing the powder into a rod and sintering this rod by an electric current in a substantial vacuum. This process, however, forms no part of the present invention, and further description of it is deemed unnecessary.

55

60

We have found that an alloy, containing 92½% of tantalum and 7½% of tungsten, is harder and stiffer than pure tantalum and at the same time provides the necessary qualities of resilience and elasticity. Alloys have been successfully used which contain as high as 10% of tungsten.

65

70

The sintered rod of the tungsten-tantalum alloy may be worked mechanically in any known manner; that is, it may be hammered, rolled, drawn, stamped and pressed in any desired form.

75

A pen may be prepared, as shown in Fig. 1, with the shank 10, the nib portion 11 and the point 12 all of the tantalum-tungsten alloy.

Although tantalum is not nearly so expensive as gold, it costs more than steel, and our invention may be applied to a modification, as illustrated in Fig. 2, where a shank 14 is of steel and is welded to the tantalum-tungsten nib 15 preferably by electrical resistance or spot welding.

80

85

In the same way the pen may be pointed with iridium, iridosmium or other tip 16 by spot welding said tip to the point of the pen.

Another method of providing a hardened tip is to merely heat the tip of the pen to a temperature above a dull red in the presence of air, hydrogen or other suitable gas. The alloy has the property of tantalum whereby this treatment makes the tip extremely hard,

90

95

and if care is used, the tip may thus be hardened without affecting the physical properties of the nib portion. A more practical and preferred method of hardening the point would be to dip the point in white hot

100 NaCO<sub>3</sub>, treat the heated tip with NaCN, or carbonize the tip in some other conventional method.

The pen prepared by using this alloy has a high degree of springiness and hardness, is one of the most resistant known to the cor-

105

rosive action of chemicals and the elements, may be manufactured as cheaply as an ordinary steel pen and will be equally as serviceable and satisfactory as the gold pen points 5 now used on fountain pens. Also by the use of the alloy defined above, a uniform product can be produced whose properties can be easily regulated to a fine degree.

While we have described particular alloys, 10 it is understood that the percentages may be varied and additional substances added to the alloy without departing from the spirit of our invention. We are not limited to the

details shown except as defined by the following claims.

15

We claim:

1. A pen having a nib comprising about 90% tantalum and 10% tungsten.
2. A pen having a nib comprising about ninety per cent tantalum and ten per cent 20 tungsten and having a hardened point.

In witness whereof, we hereunto subscribe our names this 20th day of May, 1927.

EDGAR W. ENGLE.  
MINER M. AUSTIN.